

3,340,060

**PROCESS FOR THE PRODUCTION OF COLOR IMAGES BY THE SILVER DYESTUFF BLEACHING METHOD**

Armin Meyer and René von Wartburg, Basel, and Walter Anderau, Aesch, Basel-Land, Switzerland, assignors to Ciba Limited, Basel, Switzerland, a Swiss company No Drawing. Filed Sept. 24, 1963, Ser. No. 311,235 9 Claims. (Cl. 96—53)

The present invention provides a process for the production of color photographic images by the silver dyestuff bleaching method. As is known, this method depends on the fact that dyestuffs, especially azo dyestuffs, are destroyed by a suitable treatment in the presence of metallic silver and treatment in a neutral or an acid bath containing a complex-forming agent and a bleaching catalyst. The general conception is that theoretically the bleaching of the dyestuffs proceeds stoichiometrically in accordance with the amount of silver present, four silver atoms being required to destroy one azo group. It could therefore be assumed that, in material containing a plurality of silver component images, the gradations of the color component images would depend solely upon the gradations of the developed silver images. However, this is not the case. The gradations of the color component images are dependent on many other factors, for example, on the kind of dyestuffs used, on the colloid layer, on the thickness of the layer, on the manner in which the silver is distributed within the layer, on the composition of the bleaching bath and on the duration of the bleaching process.

Proposals for independently controlling the gradations of the color component images, especially for obtaining flatter gradations, have already been made; for example, by the incorporation of non-diffusing bleaching catalysts in the light-sensitized layers, by the use of oxidizing agents in the bleaching process and by the use of several bleaching baths.

This invention is based on the surprising observation that specially advantageous effects can be obtained in the production of color photographic images by the silver dyestuff bleaching method with the aid of catalyst when the development is carried out in a bath that contains a dyestuff bleaching catalyst under conditions such that the catalyst plays no essential part in the development process.

The photographic material to be used may be, for example, material comprising a layer support, a cyan-color layer, a magenta-color layer and a yellow-color layer disposed one on top of the other in that order, each layer being made of a hydrophilic colloid such as gelatine and containing a latent silver image. The layers can also be present in the material in other sequences; the material can contain colored particles of the mixed-grain emulsion type instead of the layers; the support can be transparent or reflecting, and the material may also contain further layers, for example, adhesive layers, intermediate layers, filter layers and covering layers. This material may also contain the usual emulsion additives such as wetting agents, optical and chemical sensitizers; even small amounts of bleaching catalyst may be present in one or more layers or intermediate layers.

In the process of the invention the bath in which the latent silver image is developed contains a dyestuff bleaching catalyst. Accordingly, a proportion of the dyestuff bleaching catalyst is taken up by the layers of the photographic material being treated in the developing bath and it remains therein, at least partly, until it becomes active during the bleaching process.

The dyestuff bleaching catalysts must take no essen-

tial part in the development of the latent silver image. This can easily be arranged by using developers virtually incapable of catalyzing the dyestuff bleaching process, which is the case with most of the developers normally used. However, it is also possible to use a dyestuff bleaching catalyst that is not capable of developing a latent silver image in order to meet the requirement that the catalysts should take no essential part in the development process. It is also possible to combine the two conditions just mentioned; that is to say, the developer used is incapable of catalyzing the bleaching process and the catalyst used is incapable of developing a latent silver image.

It can easily be determined by tests whether or not developers and dyestuff bleaching catalysts meet these requirements. As an example of a developer having no catalytic action on dyestuff bleaching there may be mentioned hydroquinone, which is widely used, and which, if necessary, may be used together with other developers, for example, Metol.

As examples of dyestuff bleaching catalysts there may be mentioned phenazines, for example, 2-hydroxy-3-aminophenazine and 2:3-diaminophenazine, but more especially phenazine compounds of the formula

(1)



in which R<sub>1</sub> represents a naphthalene radical condensed with the azine ring in the manner indicated by the valence lines, which naphthalene radical contains a hydroxyl, amino and/or an azo group attached to the six-membered ring not directly bound to the azine ring, and R<sub>2</sub> represents a benzene or naphthalene radical bound to the azine ring in the manner indicated by the valence lines. Such compounds and processes for their preparation are described in U.S. patent application Ser. No. 306,690, filed Sept. 5, 1963, now U.S. Patent 3,318,700 (Swiss patent application No. 10,928/62).

Quinoxaline, alloxazine and cinnoline can also be used as dyestuff bleaching catalysts.

The process of the present invention is carried out by known methods.

The dyestuff bleaching bath comprises, as usual, an acid aqueous solution, for example, hydrochloric acid and at least one complex-forming agent, for example, potassium bromide or thiourea. This bath, too, can contain small amounts of bleaching catalyst. However, the amounts of catalyst that may be present in the material and/or in the bleaching bath must be such that they are not sufficient to bring about complete bleaching of all the color component images by the image silver present in the time available.

Accordingly, a preferred method of carrying out the process of the present invention consists in exposing in the usual manner light-sensitive multilayer material that is colored with azo dyestuffs and free from bleaching catalysts, developing it in a bath that contains a bleaching catalyst, fixing it, washing it with water, bleaching it in a bath free from catalyst, and then freeing it from residual silver in the usual manner. The fixing bath between the developing bath and dyestuff bleaching bath may be omitted.

The method can also be applied in reversal processes, the catalyst being added to the second developing bath.

In the process of the present invention the catalyst exerts a very uniform action in the various layers and exhibits favorable behaviour in respect of diffusion, so that no over-bleaching of the top layer occurs as in the usual processes.

Finally, in contrast to the processes known hitherto it is possible, in the process of the invention, to harmonize

the color gradations in such a manner that, when exposed to white light, flat color gradation curves are obtained that run parallel to one another, and that, when exposed to one spectral color, steep gradation curves are obtained. Thus, when a color chart that includes a neutral grey wedge is copied, an image is obtained in which the grey wedge is correctly reproduced and in which the colors exhibit a high degree of saturation. Should this process lead to too strong a bleaching of the lower layers, a balanced bleach can be obtained by dividing the catalyst between the developer and the dyestuff bleaching bath.

The following examples illustrate the invention. Unless otherwise stated, the parts and percentages are by weight.

#### EXAMPLE 1

The following layers are applied successively to a cellulose acetate film provided with an adhesive layer:

(1) Red-sensitive silver bromide emulsion in gelatine that contains the cyan dyestuff of the formula



(2) Gelatine intermediate layer.

(3) Green-sensitive silver bromide emulsion in gelatine that contains the magenta dyestuff of the formula



(4) Yellow filter layer that contains the dyestuff of the formula



(5) Blue-sensitive silver bromide emulsion in gelatine that contains the yellow dyestuff of the formula



and as precipitating agent a mixture comprising a reaction product of dicyanodiamidine and formaldehyde, a small amount of sodium formate and sodium bisulphite.

(6) Gelatine protective layer.

This film is exposed four times behind a grey wedge as follows:

1st exposure: in red light only

2nd exposure: in green light only

3rd exposure: in blue light only

4th exposure: in red, green and blue light the exposures being so arranged that the 4th wedge appears a neutral grey after processing.

The images obtained are designated hereinafter as "red wedge," "green wedge," "blue wedge" and "grey wedge."

The film is hardened in a formaldehyde bath, washed with water and then developed for 6 minutes in the following developer, the temperature of the developer and all subsequent baths being 24° C.

|    | Grams                              |
|----|------------------------------------|
| 10 | Sodium sulfite (anhydrous) -----   |
|    | 50                                 |
| 10 | Hydroquinone -----                 |
|    | 6                                  |
| 10 | 1-phenyl-3-pyrazolidone -----      |
|    | 0.2                                |
| 10 | Sodium carbonate (anhydrous) ----- |
|    | 35                                 |
| 10 | Potassium bromide -----            |
|    | 4                                  |
| 15 | Benztriazole -----                 |
|    | 0.3                                |
| 15 | Potassium iodide -----             |
|    | 0.05                               |
|    | Bulked with water to 1000 cc.      |

The following bleaching catalysts are added to this developer, the amounts being in milligrams per liter of developer:

#### 1st experiment

25 milligrams of 2-amino-3-hydroxyphenazine hydrochloride.

#### 2nd experiment

30 4 milligrams of 3 - (4' - sulfophenylazo) - 4 - hydroxybenzo[ $\alpha$ ]phenazine-2-sulfonic acid of the Formula 6.

#### 3rd experiment

6 milligrams of 3-amino-4-hydroxybenzo[ $\alpha$ ]phenazine-2-sulfonic acid of the Formula 7.

The film is then treated in the following stop fixation bath without an intermediate wash with water:

|    |                               |       |    |
|----|-------------------------------|-------|----|
| 45 | Sodium acetate -----          | grams | 10 |
|    | Thiourea -----                | do    | 50 |
|    | Glacial acetic acid -----     | cc    | 20 |
|    | Bulked with water to 1000 cc. |       |    |

The film is washed with water for 3 minutes and then



bleached in a dyestuff bleaching bath having the following composition:

|    |                                                                                                                   |       |     |
|----|-------------------------------------------------------------------------------------------------------------------|-------|-----|
| 65 | Potassium bromide -----                                                                                           | grams | 100 |
|    | Thiourea -----                                                                                                    | do    | 10  |
|    | Hydrochloric acid (conc.) -----                                                                                   | cc    | 70  |
|    | 1.25% aqueous solution of the addition product of 35 mols of ethylene oxide with 1 mol of octadecyl alcohol ----- | cc    | 10  |
|    | Bulked with water to 1000 cc.                                                                                     |       |     |

The time of treatment in this bath is so selected that it is just sufficient to bring about complete bleaching of the dyestuffs in all layers at the places most highly exposed,

the said time of treatment having been determined by tests. It is as follows:

|                | Minutes |
|----------------|---------|
| 1st experiment | 8       |
| 2nd experiment | 15      |
| 3rd experiment | 15      |

The film is then washed with water, the residual silver rehalogenated in a copper nitrate bath made strongly acid with hydrochloric acid, washed again, fixed, washed and then dried.

When repeating these experiments but omitting the bleaching catalyst in developer I, only a very slight degree of dyestuff bleaching is obtained.

In three further experiments the same procedure as above is adopted but omitting the developers 1-phenyl-3-pyrazolidone and hydroquinone in developer I. In this process no silver image is visible before the bleaching bath; on completion of the process no bleaching of the dyestuffs is observed.

The dyestuff in the blue-sensitive layer can be prepared by diazotizing 2-aminonaphthalene-4:8-disulfonic acid, coupling the diazo compound with 1-amino-2-methylbenzene, and treating the aminomonoazo dyestuff so obtained with phosgene.

The catalyst 3-(4'-sulfonylazo)-4-hydroxybenzo[ $\alpha$ ]phenazine-2-sulfonic acid of the formula



is obtained by coupling diazotized 1-aminobenzene-4-sulfonic acid with 4-hydroxybenzo[ $\alpha$ ]phenazine-2-sulfonic acid, which acid is obtained by cyclizing the product obtained by coupling diazotized 1-aminobenzene-4-sulfonic acid with 2-phenylamino-5-hydroxynaphthalene-7-sulfonic acid.

The catalyst 3-amino-4-hydroxybenzo[ $\alpha$ ]phenazine-2-sulfonic acid of the formula

(7)



is obtained from the foregoing catalyst by splitting the azo group with sodium hydrosulfite.

#### EXAMPLE 2

The experiments described in Example 1 are repeated using the following developer II:

|                               | Grams |
|-------------------------------|-------|
| Metol                         | 2.5   |
| Sodium sulfite (anhydrous)    | 30    |
| Hydroquinone                  | 2.5   |
| Sodium metaborate             | 10    |
| Potassium bromide             | 0.5   |
| Bulked with water to 1000 cc. |       |

The following bleaching catalysts are added to this developer, the amounts being in milligrams per liter of developer:

75

#### 1st experiment

4 milligrams of 2-amino-3-hydroxyphenazine hydrochloride.

#### 2nd experiment

4 milligrams of 2-amino-3-hydroxyphenazine hydrochloride.

4 milligrams of 3-(4'-sulfonylazo)-4-hydroxybenzo[ $\alpha$ ]phenazine-2-sulfonic acid of the Formula 6.

10

#### 3rd experiment

4 milligrams of 2-amino-3-hydroxyphenazine hydrochloride.

15

4 milligrams of 3-amino-4-hydroxybenzo[ $\alpha$ ]phenazine-2-sulfonic acid of the Formula 7.

20

The developing time is 8 minutes. The time of treatment in the dyestuff bleaching bath which is just sufficient to bring about complete bleaching of the dyestuffs in all layers

25

at the areas most highly exposed is as follows:

|                | Minutes |
|----------------|---------|
| 1st experiment | 10      |
| 2nd experiment | 10      |
| 3rd experiment | 12      |

25

Only a very slight degree of bleaching is achieved when the bleaching catalyst is omitted in developer II. No silver image is visible and no dyestuff bleaching takes place when the two developers Metol and hydroquinone are omitted in developer II.

#### EXAMPLE 3

A film of the composition given in Example 1 is exposed, hardened in a formaldehyde bath, washed with water and then developed for 4 minutes in developer I, which developer contains 30 milligrams of 2-amino-3-hydroxyphenazine hydrochloride per liter as bleaching catalyst. The film is washed with water for 2 minutes and then treated for 4 minutes in the dyestuff bleaching bath

35 as described in Example 1 which is free from bleaching catalyst. In accordance with Example 1, the residual silver is then rehalogenated and fixed. The time of treatment in the dyestuff bleaching bath is so selected that it is just sufficient to bring about complete bleaching of the dyestuffs in all layers at the areas most highly exposed, which

40 time is determined by experiment.

45 For comparison purposes, a series of 4 exposures produced in the same manner as above is subjected to the same treatment, with the exception that the developer I is free from bleaching catalyst and the same catalyst was

50 added to the dyestuff bleaching bath in an amount of 2 milligrams per liter. The minimum time required to bring about complete bleaching is 8 minutes.

The results obtained in the two experiments in respect 55 of gradation (gamma value) and extent of exposure are listed in the following table, the extent of exposure being designated with  $\Delta \log E$ .

$$\Delta \log E = \log E_{\max} - \log E_{\min}$$

60 whereby  $E_{\max}$  and  $E_{\min}$  represent the strongest and weakest exposures respectively that are capable of being copied. The color densities are measured with a Macleth-Ansco-Densitometer in transmitted light; the gamma values correspond to the straight parts of the gradation curves.

| Designation of wedge | Measuring filter | Catalyst in developer |                 | Catalyst in dyestuff bleaching bath |                 |
|----------------------|------------------|-----------------------|-----------------|-------------------------------------|-----------------|
|                      |                  | Gamma                 | $\Delta \log E$ | Gamma                               | $\Delta \log E$ |
| Grey wedge           | Red              | 0.5                   | 1.8             | 0.6                                 | 1.5             |
|                      | Green            | 1.1                   | 1.8             | 1.2                                 | 1.5             |
|                      | Blue             | 0.9                   | 1.9             | 1.1                                 | 1.6             |
| Red wedge            | Red              | 0.7                   | 1.4             | 0.7                                 | 1.2             |
| Green wedge          | Green            | 1.0                   | 1.4             | 1.0                                 | 1.2             |
| Blue wedge           | Blue             | 0.6                   | 1.9             | 0.8                                 | 0.6             |

## EXAMPLE 4.

Multi-layer silver dyestuff bleaching material cast on baryta paper and hardened while casting, but otherwise having the same composition as in Example 1 is exposed and developed. The silver is converted into silver chloride in a bleaching bath and the resulting chloride dissolved out selectively. The silver bromide that remains is exposed in diffused light and developed for 10 minutes in a developer having the following composition:

|                               |            |     |
|-------------------------------|------------|-----|
| Water                         | cc         | 750 |
| Sodium sulfite (anhydrous)    | grams      | 50  |
| 1-phenyl-3-pyrazolidone       | do         | 0.2 |
| Hydroquinone                  | do         | 6   |
| Sodium carbonate (anhydrous)  | do         | 35  |
| Potassium bromide             | do         | 2   |
| Sodium thiocyanate            | do         | 2   |
| Thallium nitrate              | milligrams | 50  |
| Bulked with water to 1000 cc. |            |     |

This solution also contains 25 milligrams of the dyestuff bleaching catalyst 3-amino-4-hydroxybenzo[ $\alpha$ ]phenazine-2-sulfonic acid of the Formula 7.

The layer is then washed with water for 1 minute and bleached for 8 minutes in a bath having the following composition:

|                                        |             |     |
|----------------------------------------|-------------|-----|
| Water                                  | millimeters | 750 |
| Potassium bromide                      | grams       | 100 |
| Hydrochloric acid (37% strength)       | millimeters | 70  |
| Thiourea                               | grams       | 10  |
| Bulked with water to 1000 millimeters. |             |     |

This bath also contains 1 milligram of the dyestuff bleaching catalyst 3-(4'-sulfophenylazo)-4-hydroxybenzo[ $\alpha$ ]phenazine-2-sulfonic acid of the Formula 6.

The layer is washed with water and the excess silver converted into silver chloride in known manner with the aid of a copper-containing bleaching bath, and the chloride dissolved out in a subsequent fixing bath. The resulting color image exhibits high color densities at the highly exposed areas after the above treatment, and the dyestuffs are bleached out at the areas of low exposure.

## EXAMPLE 5

A silver bromide-silver iodide emulsion that contains the black dyestuff of the formula



and a hardening agent is cast on to a photographic paper.

A sheet of type-written paper is brought into contact with the said photographic paper in such a manner that the back of the original lies on the photographic layer. The composite specimen is exposed for 15 seconds in a photocopying apparatus of conventional design, and the layer developed in a Metol-hydroquinone rapid developer that contains 100 cc. of a solution of 1% 2:3-dimethylquinoxaline in isopropanol in 1000 cc. of developer. The layer is then introduced into a dyestuff bleaching bath that contains, per 1000 cc. of water, 50 grams of thiourea, 100 grams of potassium bromide and 100 cc. of 37% hydrochloric acid. A positive image of the original is formed after 2 minutes. The excess silver is subsequently removed with the aid of a normal bleach fixation bath.

When the 2:3-dimethylquinoxaline solution is omitted from the developer, no dyestuff bleaching takes place and a completely black sheet of paper is obtained.

What is claimed is:

1. In a process for the production of color photographic

images by the silver dyestuff bleaching method with the aid of catalysts, the step which comprises carrying out the development in a bath that contains a dyestuff bleaching catalyst and under conditions such that the catalyst plays no essential part in the development process.

2. In a process for the production of color photographic images by the silver dyestuff bleaching method with the aid of catalysts, the step which comprises carrying out the development in a bath that contains a developer not capable of catalyzing the dyestuff bleaching process and also a dyestuff bleaching catalyst.

3. In a process for the production of color photographic images by the silver dyestuff bleaching method with the aid of catalysts, the step which comprises carrying out the development in a bath that contains a developer not capable of catalyzing the dyestuff bleaching process and also a dyestuff bleaching catalyst not capable of developing a latent silver image.

4. In a process for the production of color photographic images by the silver dyestuff bleaching method with the aid of catalysts, the step which comprises carrying out the development in a bath that contains a developer not capable of catalyzing the dyestuff bleaching process and also a phenazine as a dyestuff bleaching catalyst.

5. In a process for the production of color photographic images by the silver dyestuff bleaching method with the aid of catalysts, the step which comprises carrying out the development in a bath that contains a developer not capable of catalyzing the dyestuff bleaching process and also a quinoxaline as a dyestuff bleaching catalyst.

6. In a process for the production of multi-color photographic images by the silver dyestuff bleaching method with the aid of catalysts, the step which comprises carrying out the development in a bath that contains hydroquinone as a developer and also a phenazine as a dyestuff bleaching catalyst.

7. In a process for the production of multi-color photographic images by the silver dyestuff bleaching method with the aid of catalysts, the step which comprises carrying out the development in a bath that contains hydroquinone as a developer and also 2-amino-3-hydroxyphenazine as a dyestuff bleaching catalyst.

8. In a process for the production of multi-color photographic images by the silver dyestuff bleaching method with the aid of catalysts, the step which comprises carry-

ing out the development in a bath that contains hydroquinone as a developer and also 3-(4'-sulfophenylazo)-4-hydroxybenzo[ $\alpha$ ]phenazine-2-sulfonic acid as a dyestuff bleaching catalyst.

9. In a process for the production of multi-color photographic images by the silver dyestuff bleaching method with the aid of catalysts, the step which comprises carrying out the development in a bath that contains hydroquinone as a developer and also 3-amino-4-hydroxybenzo[ $\alpha$ ]phenazine-2-sulfonic acid as a dyestuff bleaching catalyst.

## References Cited

## UNITED STATES PATENTS

|           |         |               |       |
|-----------|---------|---------------|-------|
| 2,004,625 | 6/1935  | Gasper        | 96-53 |
| 2,221,793 | 11/1940 | Gasper        | 96-53 |
| 2,278,984 | 4/1942  | Gasper et al. | 96-53 |
| 3,156,561 | 11/1964 | Dreyfuss      | 96-20 |
| 3,278,303 | 10/1966 | Meyer et al.  | 96-53 |

UNITED STATES PATENT OFFICE  
CERTIFICATE OF CORRECTION

Patent No. 3,340,060

September 5, 1967

Armin Meyer et al.

It is hereby certified that error appears in the above numbered patent requiring correction and that the said Letters Patent should read as corrected below.

In the heading to the printed specification, after line 8, insert -- Claims priority, application Switzerland, Oct. 5, 1962, 11760/62 --.

Signed and sealed this 22nd day of October 1968.

(SEAL)

Attest:

Edward M. Fletcher, Jr.

Attesting Officer

EDWARD J. BRENNER

Commissioner of Patents